

## UNITED STATES PATENT OFFICE

2,671,029

## PORCELAIN ENAMELING

Le Roy L. Moss, Cleveland, Ohio, assignor to  
Ferro Corporation, a corporation of OhioNo Drawing. Application May 14, 1951,  
Serial No. 226,273

10 Claims. (Cl. 106—48)

**1**  
This invention relates as indicated to porcelain enameling and has more particular reference to dry-milled enamels and to a process for producing the same.

In the present day practice of dry-milling porcelain enamel, the frit is placed in a dry mill with grinding balls and then ground until about 97% passes through a 200 mesh sieve. This finely ground material is then either fired directly on cast iron (dry process) or it is blunged with water, clay, salts etc. and then applied to sheet steel (wet process).

Porcelain enamels bearing antimony or zirconia as the opacifying agent when used in dry-milling applications are particularly troublesome. These enamels when dry-ground and applied by either the wet or dry process and then fired onto a work piece cause the finished piece to be disfigured by the presence of minute black specks scattered throughout the surface.

It is, therefore, the principal object of this invention to provide a process whereby dry-milled antimony and zirconia porcelain enamels will produce a surface on a work piece which is substantially entirely free of black specks.

Other objects will become apparent as the description proceeds.

To the accomplishment of the foregoing and related ends, the invention, then, comprises the features hereinafter fully described and particularly pointed out in the claims, the following description setting forth in detail certain illustrative embodiments of the invention, these being indicative, however, of but a few of the various ways in which the principle of the invention may be employed.

Broadly stated this invention comprises the process of producing dry-milled porcelain enamel frits which upon subsequent firing onto a work piece are substantially free of black specks which comprises charging a mill with a frit selected from the class consisting of antimony-opacified frits or zirconia-opacified frits, adding a minor amount of a carbon dioxide-absorbing agent and milling said frit and carbon dioxide-absorbing agent.

After extensive study I have evolved the theory that black specks develop on dry-milling because of carbon dioxide pick-up of the finely divided material in the presence of moisture. I have found that by adding small amounts of such carbon dioxide-absorbing agents as the hydroxides of sodium, potassium and magnesium to the mill containing the porcelain enamel frit the resultant ground material shows substantially no

**2**  
black-specking when fired on a work piece. I have also found that various commercial carbon dioxide-absorbing agents such as "Garoxite" and "Ascarite" function efficiently in the prevention of black-specking in the porcelain enamels. These commercial carbon dioxide-absorbing agents are substantially sodium hydrate admixed with asbestos.

I have also discovered that, while the carbon dioxide-absorbing agents prevent black-specking the addition of small amounts of a water-repellent, such as the General Electric "Dri-Films" which are organochlorosilanes, enhance the lasting effects of the CO<sub>2</sub>-absorbing agent. I have found that by adding from about 0.025% to about 0.3% of methylchlorosilane in addition to the CO<sub>2</sub>-absorbing agent the milled porcelain enamel can be left to stand for long periods without picking up moisture and therefore will not black speck when fired on a work piece.

It is to be noted that while the CO<sub>2</sub>-absorbing agents function alone to prevent black-specking the water-repellent agent alone will not prevent the black-specking.

**25** In the preferred embodiment of my invention I use from about  $\frac{1}{8}$ % to about 2% CO<sub>2</sub>-absorbing agents per 100 parts of frit and from about 0.025% to about 0.3% of an organochlorosilane per 100 parts of frit.

**30** When I refer to an antimony or a zirconia-opacified frit I am referring to a frit to which the antimony and zirconia have been added as a smelter addition. The following formulae are typical examples of what is meant by frits which contain antimony and zirconia as the opacifying agents. These formulae are just two examples of many possible variations which exist. However, any formulations which contain antimony and zirconia as the opacifying agents are applicable to the present invention.

## I. Antimony-opacified formula

|                  | Pounds |
|------------------|--------|
| 45 Silica sand   | 601    |
| Dehydrated borax | 318    |
| Feldspar         | 657    |
| Antimony oxide   | 188    |
| Soda ash         | 58     |
| Soda nitrate     | 81     |
| 50 Fluorspar     | 111    |
| Cryolite         | 372    |
| Zinc oxide       | 54     |
| Barium carbonate | 42     |

## 3

## II. Zirconia-opacified formula

|                      | Pounds |
|----------------------|--------|
| Silica sand          | 57     |
| Dehydrated borax     | 363    |
| Feldspar             | 498    |
| Zircon sand          | 386    |
| Fluorspar            | 91     |
| Sodium-fluo-silicate | 325    |
| Bone ash             | 106    |
| Aluminum hydrate     | 98     |
| Zinc oxide           | 53     |

Of course my invention works equally well where antimony and zirconia have been added to the mill besides being present as smelter components.

A typical procedure in following the process of my invention would be to add about 1% of magnesium hydroxide and about 0.125% of an organochlorosilane per 100 parts of antimony or zirconia-opacified frit to a dry mill and then grinding until at least 60% of the frit passes through a 200 mesh sieve. It is to be noted that the final particle size of the milled frit is determined by its end use. That is whether it is to be used on cast iron or sheet steel or used as a dry process application or a wet process application. Those skilled in the art will readily recognize the proper particle size according to their use and method of application.

Other modes of applying the principle of the invention may be employed provided the features stated in any of the following claims or the equivalent of such be employed.

I therefore particularly point out and distinctly claim as my invention:

1. The method of producing dry-milled porcelain enamels frits which upon subsequent firing onto a work piece are substantially free of black specks which comprises charging a mill with a frit selected from the class consisting of antimony-opacified and zirconia-opacified frits adding from about 1/8% to about 2% per 100 parts of said frit of a carbon dioxide-absorbing agent and then milling said mixture until at least 60% of said mixture passes through a 200 mesh sieve.

2. The method of producing dry-milled porcelain enamels frits which upon subsequent firing onto a work piece are substantially free of black specks which comprises charging a mill with a frit selected from the class consisting of antimony-opacified and zirconia-opacified frits adding from about 1/8% to about 2% per 100 parts of said frit of a carbon dioxide-absorbing agent and from about 0.025% to about 0.3% of an organochlorosilane and then milling said mixture until at least 60% of said mixture passes through a 200 mesh sieve.

3. The method of producing dry-milled porcelain enamels frits which upon subsequent firing onto a work piece are substantially free of black specks which comprises charging a mill with a frit selected from the class consisting of antimony-opacified and zirconia-opacified frits adding from about 1/8% to about 2% per 100 parts of said frit of sodium hydroxide and from about 0.025% to about 0.3% of an organochloro-

silane and then milling said mixture until at least 60% of said mixture passes through a 200 mesh sieve.

4. The method of producing dry-milled porcelain enamels frits which upon subsequent firing onto a work piece are substantially free of black specks which comprises charging a mill with a frit selected from the class consisting of antimony-opacified and zirconia-opacified frits adding from about 1/8% to about 2% per 100 parts of said frit of potassium hydroxide and from about 0.025% to about 0.3% of an organochlorosilane and then milling said mixture until at least 60% of said mixture passes through a 200 mesh sieve.

5. The method of producing dry-milled porcelain enamels frits which upon subsequent firing onto a work piece are substantially free of black specks which comprises charging a mill with a frit selected from the class consisting of antimony-opacified and zirconia-opacified frits adding from about 1/8% to about 2% per 100 parts of said frit of magnesium hydroxide and from about 0.025% to about 0.3% of an organochlorosilane and then milling said mixture until at least 60% of said mixture passes through a 200 mesh sieve.

6. A new composition of matter comprising a dry-milled frit selected from the class of antimony and zirconia-opacified frits, and from about 1/8% to about 2% of a carbon dioxide-absorbing agent per 100 parts frit.

7. A new composition of matter comprising a dry-milled frit selected from the class of antimony-opacified and zirconia-opacified frits from about 1/8% to about 2% of a carbon dioxide-absorbing per 100 parts frit and from about 0.025% to about 0.3% of an organochlorosilane per 100 parts frit.

8. A new composition of matter comprising a dry-milled frit selected from the class of antimony-opacified and zirconia-opacified frits from about 1/8% to about 2% of sodium hydroxide per 100 parts frit and from about 0.025% to about 0.3% of an organochlorosilane per 100 parts frit.

9. A new composition of matter comprising a dry-milled frit selected from the class of antimony-opacified and zirconia-opacified frits from about 1/8% to about 2% of potassium hydroxide per 100 parts frit and from about 0.025% to about 0.3% of an organochlorosilane per 100 parts frit.

10. A new composition of matter comprising a dry-milled frit selected from the class of antimony-opacified or zirconia-opacified frits from about 1/8% to about 2% of magnesium hydroxide per 100 parts frit and from about 0.025% to about 0.3% of an organochlorosilane per 100 parts frit.

LE ROY L. MOSS.

References Cited in the file of this patent

UNITED STATES PATENTS

Number Name Date  
 2,090,617 Bley Aug. 24, 1937  
 2,556,896 Beatty et al. June 12, 1951